

Sept. 5, 1944.

C. E. McMANUS ET AL

2,357,416

CAP

Filed July 25, 1940

Fig. 1.



Fig. 2.



Inventor

Charles E. McManus.  
Giles B. Cooke.

By *Cushman Daily & Cushman*  
Attorneys

## UNITED STATES PATENT OFFICE

2,357,416

## CAP

Charles E. McManus, Spring Lake, N. J., and Giles B. Cooke, Baltimore, Md., assignors to Crown Cork & Seal Company, Inc., Baltimore, Md., a corporation of New York

Application July 25, 1940, Serial No. 347,538

1 Claim. (Cl. 215—39)

This invention relates to closures of the skirted type having a cushion liner disposed therein.

The cap of the present invention is provided with a protective coating applied by a single operation as by spraying on the surface of the cushion liner and the adjacent interior wall of the cap skirt including the raw edge thereof. This continuous facing, when the cap is sealed upon a container, is interposed between the contents and the cushion liner and acts in a manner similar to center spots and overall facings of paper and foil which have heretofore been used. Moreover, the coating on the inner wall of the cap skirt and particularly the raw or free edge thereof not only assures additional rustproofness, but effectively closes any pores or bruised or otherwise uncovered portions in the lacquer surface of the cap.

A particularly important feature of the invention resides in forming the continuous film on the interior exposed surface of an assembled cap, i. e., shell with liner therein, by a single operation. We have found by spraying a solution of protective material into the interior of the assembled cap, that on drying, a thin continuous film is produced coextensive with both the area of the liner and the entire exposed area of the skirt including its raw edge. Caps having the novel construction of this invention are thus cheaply and rapidly produced.

Before describing in detail the present invention, it is to be understood that the invention is not limited in its application to the details of construction and arrangements of parts illustrated in the accompanying drawing, since the invention is capable of other embodiments and of being practiced or carried out in various ways. Also, it is to be understood that the phraseology or terminology employed herein is for the purpose of description and not of limitation, and it is not intended to limit the invention claimed herein beyond the requirements of the prior art.

In the drawing,

Figure 1 is a sectional view showing a crown cap provided with a protective film in accordance with this invention; and

Figure 2 is a bottom elevation of a crown cap.

Referring to Figure 1, there is shown for purposes of illustration a metal crown cap having a top 10 and a depending crimped skirt 11. The invention may be employed with any desired skirted closure, for example, a screw cap, a lug cap, or a pressed-on cap. The cap shell is customarily coated with a suitable protective lac-

quer both interiorly and exteriorly, and there is assembled within the shell a cushion liner 12 united thereto by a suitable adhesive. This cushion liner is composed of various materials such as paper, rubber, natural or composition cork. Cork liners are most generally used.

The continuous protective film in accordance with this invention is of a thickness about substantially five ten thousandths to three thousandths of an inch, and is indicated at 13. It constitutes a continuous, adherent facing upon the exposed surface of the liner 12 and the adjacent interior wall of the cap skirt including its raw or free edge 14. In the case of caps such as crown caps, lug caps and screw caps, or other skirted closures in which the skirt has an irregular contour, the film is coextensive with and adhered to the entire exposed surface of the interior of the cap. That is to say, in crown caps for example, the film covers the cushion liner and extends integrally therefrom to continuously cover both the hills and valleys of the crimped or corrugated area and the raw edge.

As explained above, the facing layer on the liner serves the purpose of the more expensive adhered facings of paper or foil, and its presence on the skirt and raw edge assure enhanced rustproofness and complete coverage of any bruised areas, pores, or uncovered portions in the lacquered surface of the crown.

The protective material employed is one which is adherent to metal, the lacquer coating, and the composition liner. It also has the necessary resistant properties so that it will not react with the contents such as beverages and foods and will impart rustproofness and abrasion resistance to the cap shell, particularly at the raw edge of the same. Preferably, dilute solutions of the film forming material are employed, e. g., 2 to 10 percent solutions in a suitable low boiling solvent, but greater concentrations may be used in some cases, e. g., up to 30% dependent upon the nature of the coating materials. We prefer to use substances such as "Vinylite" resin, chlorinated rubber, polyvinyl acetal resin and ethyl cellulose, but numerous other odorless and tasteless coating materials which likewise form a transparent coating and have the required properties may be used.

By way of example, suitable solutions comprise 5 percent "Vinylite" resin in acetone; a 5 percent solution of chlorinated rubber in chloroform; and a 5 percent solution of polyvinyl acetal resin in ethylene dichloride, and a 5 percent solution of ethyl cellulose in chloroform.

Of particular importance, the film is applied effectively to assure rapid and inexpensive manufacture by spraying one of the solutions above mentioned upon the interior of the cap. In other words, in a single operation upon the assembled cap, i. e., the cap shell and liner therein, we are able to produce the continuous facing film of the same material on the liner and on the adjacent inner wall of the cap skirt including its raw edge. We prefer to accomplish the operation by spraying, but satisfactory results may be obtained by brushing the solution upon the interior of the assembled cap or by dipping the cap in the solution.

After the solution has been applied to the cap, the protective film is deposited from the solution by drying, care being taken to remove all traces of solvent.

In some cases, as where the film 13 lacks complete continuity between the cushion liner 12 and the interior wall surface of the cap, when the cap such as a crown is crimped upon the sealing lip of the container, the adjacent surfaces of the liner and skirt are brought together so that the coating 13 for all practical purposes, has the form of the originally sprayed continuous film as shown in Figure 1. In any case, the protective film is coextensively adhered to

both the sealing liner and the adjacent exposed surface of the cap skirt including the raw edge thereof, and thereby a continuous coating is produced which bridges the joint between the sealing liner and the cap skirt, as shown in Fig. 1.

The provision of the film forming protective materials above described is particularly advantageous with certain types of cushion liners such as those made of newsboard or paper pulp having the conventional glazed paper facing. These are relatively hard as compared to cork or cork composition, and the film being tough, compressible and resilient substantially assists in forming an effective seal between the cap and the sealing lip of the container.

We claim:

A cap having a top and a skirt, a cushion liner within the cap, and a protective film coextensively coated and adhered on the exposed surface of the liner and the entire adjacent interior exposed surface of the cap skirt including the raw edge thereof, the film on the liner and the film on the skirt being of the same material and continuous with each other and bridging the joint between the cushion liner and the cap skirt.

CHARLES E. McMANUS.  
GILES B. COOKE.